

# UNITED STATES PATENT OFFICE.

MYRTIL KAHN, OF ELBERFELD, GERMANY, ASSIGNOR TO FARBENFABRIKEN OF ELBERFELD CO., OF NEW YORK, N. Y., A CORPORATION OF NEW YORK.

## PROCESS OF DYEING.

SPECIFICATION forming part of Letters Patent No. 725,847, dated April 21, 1903.

Application filed January 27, 1903. Serial No. 140,720. (No specimens.)

To all whom it may concern:

Be it known that I, MYRTIL KAHN, doctor of philosophy, chemist, residing at Elberfeld, Germany, (assignor to the FARBENFABRIKEN OF ELBERFELD CO., of New York,) have invented a new and useful Improvement in Processes of Dyeing; and I do hereby declare the following to be an exact and clear description of my invention.

10 I have found that black shades of great fastness can be obtained on dyeing wool with certain azo dyestuffs derived from ortho-amidophenol derivatives and on treating the dyed goods with chromium compounds react-  
15 ing as oxidizing agents, such as chromates, bichromates, or the like. By the action of these chromium compounds the original shades varying from red to blue are changed into deep-black shades, distinguished for  
20 their fastness to the "potting process," which is a finishing process for woolen piece goods. In this process the goods are entered into boiling water and allowed to remain there until the water is cold. The goods thus as-  
25 sume a high degree of gloss and softness, and, according to the effect desired, the "potting" may be repeated several times. They also resist milling and washing and possess great fastness against the action of light. The col-  
30 oring-matters which I use for this purpose can be prepared by combining the diazo com-  
pounds of o-amidophenol derivatives having the following general formula:



X meaning  $-\text{SO}_3\text{H}$ ;  $-\text{COOH}$  or  $-\text{CH}_2\text{SO}_3\text{H}$ ; Y meaning a hydrogen atom which can be replaced by  $-\text{CH}_3$ ; -halogen;  $-\text{NO}_2$  or  $-\text{SO}_3\text{H}$ , such as o-amidophenol sulfonic acids, amidoxybenzoic acids, or amidoxybenzyl sulfonic acids (containing the amido and the hydroxy group in ortho position) or

derivatives thereof—such as amidocresol sul- 45 fonic acids, the sulfonic acids of o-amido-  
salicylic acid, or the halogenated or nitrated derivatives of all these compounds, with 1:5  
dioxynaphthalene having the formula:



In carrying out my process practically I can proceed as follows: Place the wool in a bath containing three to six per cent. sul- 60 furic acid, ten per cent. Glauber's salt, and six per cent. of the dyestuff prepared by combination of diazotized ortho-amidophenol-  
65 para-sulfonic acid with 1:5 dioxynaphthalene, bring slowly to boil and boil for forty-  
five minutes. The reddish-violet shade thus obtained is changed into deep black by boiling the dyed wool for one-half hour in a bath containing three to four per cent. bichromate 70 of potash and three to six per cent. sulfuric acid. For the treatment with the above-mentioned chromium compounds the old dye-  
75 bath can also be used. In this case the further addition of sulfuric acid is not necessary.

The process proceeds in an analogous manner on using other of the above-cited dyestuffs or other chromium compounds reacting as oxidizing agents. Of course instead of sulfuric acid another suitable acid may be 80 used, such as acetic acid or the like.

Having now described my invention and in what manner the same is to be performed, what I claim as new, and desire to secure by Letters Patent, is—

85 The herein-described process for producing on wool fast-black shades, which process consists in first dyeing wool from acid-bath with

dyestuffs obtainable by combination of the diazo derivatives of o-amidophenol derivatives having the above-given general formula with 1:5 dioxy naphthalene and then treating  
5 the dyed goods with chromium compounds reacting as oxidizing agents, substantially as described.

In testimony whereof I have signed my name in the presence of two subscribing witnesses.

MYRTIL KAHN.

Witnesses:

OTTO KÖNIG,  
T. A. RITTERSHAUS.